

# UNITED STATES PATENT OFFICE.

WILLIAM G. LINDSAY, OF NEW YORK, N. Y., ASSIGNOR TO THE CELLULOID COMPANY,  
A CORPORATION OF NEW JERSEY.

## NON-INFLAMMABLE ACETYL-CELLULOSE COMPOSITION.

1,133,385.

Specification of Letters Patent. Patented Mar. 30, 1915.

No Drawing.

Application filed May 5, 1909. Serial No. 494,180.

To all whom it may concern:

Be it known that I, WILLIAM GODSON LINDSAY, a citizen of the United States, residing at New York city, in the county of 5 New York and State of New York, have invented certain new and useful Improvements in Non-Inflammable Acetyl-Cellulose Compositions, of which the following is a full, clear, and exact specification.

10 This invention relates to improvements in non-inflammable photographic films, and relates to a non-inflammable transparent composition of matter containing an organic esterified compound of cellulose such as 15 acetyl cellulose, and particularly adaptable to be made in the form of thin sheets or films for photographic and similar purposes.

More particularly my invention relates to 20 a film containing an acetyl cellulose compound in combination with substances for effecting non-inflammability and permanency of strength and tenacity.

Films containing nitro-cellulose have had 25 extensive use as applied to photographic plates or as films, and especially in the form of long strips which bear photographic prints in what is known as the cinematograph apparatus. The high inflammability 30 of nitro-cellulose films has called for a substitute that would be less hazardous in operating cinematograph and similar apparatus. Heretofore, it has been proposed to form films of substances other than nitro-cellulose, but such films have presented several objections, so that for practical purposes the nitro-cellulose film is still preferred to such substitutes. These prior substitutes have a tendency to harden or become 40 brittle, and so far as I am aware of none is non-inflammable. The thin sheet or strip of film made in accordance with my invention is free from all danger of inflammability or ignition, and in addition is transparent and possesses permanently a high degree of strength and tenacity.

In carrying out my invention I may take 50 any acetyl cellulose which is soluble in acetone to which has been added triphenyl-phosphate as hereinafter described. The amount of acetone, which has a relatively low boiling point of 58° C. employed depends upon the consistency desired for spreading the solution upon glass or other

smooth surface. To this solution I may add 55 suitable quantities of a restraining agent, such as acetylene tetrachlorid, which has a relatively high boiling point of 147° C. or equivalent substance. The film or strip may now be formed by spreading the solution 60 upon any smooth surface, such as glass. The solvents are now allowed to evaporate in the usual way, which results in leaving a dried and hardened film or strip. The acetone, or low boiling solvent, evaporates from 65 the film in a comparatively short time, but the evaporation of the acetylene tetrachlorid, or high boiling solvent, proceeds more slowly, and a very long time may elapse 70 before there is substantially complete evaporation thereof. The film, however, will be dry and hard enough for use in a very considerable time before the high boiling solvent has substantially evaporated.

The product obtained by following the 75 above mentioned steps possesses great strength and tenacity, is transparent and is substantially non-inflammable. The triphenylphosphate produces a decided strengthening and non-inflammable effect. 80 To render permanent the strength and tenacity of the product urea in proper proportions may be employed in addition to the triphenylphosphate.

I have found the following ingredients 85 with the proportions as indicated to give most excellent results:

### Parts by weight.

|                        |     |    |
|------------------------|-----|----|
| Acetyl cellulose       | 100 | 90 |
| Acetone                | 300 |    |
| Triphenylphosphate     | 15  |    |
| Acetylene tetrachlorid | 45  |    |
| Urea                   | 2   |    |

It will be understood that the product 95 formed in accordance with this invention is not limited to the exact proportions set forth above, and that my invention is not limited to the specific substances as indicated. Any acetyl cellulose which is soluble 100 in a menstruum in the presence of triphenyl-phosphate, or equivalent substance is suitable. The acetone ingredient may be replaced in part or in whole by any suitable solvent. The acetylene tetrachlorid may be 105 replaced entirely or in part by equivalent substances. The degree of thinness of the film will control to some extent the extreme

proportions of the substances used to obtain my product. A 10-part proportion of triphenylphosphate gives a satisfactory strength and produces a substantially non-inflammable product; in extremely thin films it might be found desirable to raise the proportion, say to 25 parts. A very small proportion of urea will prevent or retard the tendency to become brittle, so that 10 for many purposes the proportion need not be two per cent.

The invention set forth in this application is of special utility as a film or plate for photographic purposes, both as negatives and as positives, and particularly in 15 the form of long strips for use in cinematograph and similar apparatus. The film made in accordance with this invention is highly flexible and possesses unusual 20 strength, and will not burn with a self-sustaining flame even when the film hangs pendant. It is to be noted that the qualities of strength and pliability of my product are permanent in character, and are capable 25 of receiving and retaining sensitized emulsion for use in photographic processes.

Having thus described my invention, I declare that what I claim as new and desire to 30 secure by Letters Patent, is—

30 1. A product comprising an organic esterified compound of cellulose and triphenylphosphate obtained by dissolving the same in a solvent common to both, and then permitting the solution to dry and harden 35 by evaporation.

2. A product comprising an organic acid ester of cellulose and triphenylphosphate obtained by dissolving the same in a solvent common to both, and then permitting the 40 solution to dry and harden by evaporation.

3. A product comprising an organic esterified compound of cellulose and a noninflammable material which is insoluble in water, obtained by dissolving the same in a 45 solvent common to both and a fluid restrain-

ing agent, and then permitting the solution to dry and harden by evaporation.

4. A product comprising an organic esterified compound of cellulose and triphenylphosphate obtained by dissolving the same in a solvent common to both, to which solvent has been added a fluid restraining agent and then permitting the solution to dry and harden by evaporation.

5. A product comprising an acetyl cellulose and triphenylphosphate obtained by dissolving the same in a mixture of acetone and acetylene tetrachlorid, and then permitting the solution to dry and harden by evaporation.

6. A product comprising an acetyl cellulose and triphenylphosphate obtained from dissolving the same in a solvent common to both, to which has been added a fluid restraining agent, and then permitting the 65 same to dry and harden by evaporation.

7. A product comprising acetyl cellulose and triphenylphosphate obtained by dissolving the same in acetone, and then permitting the solution to dry and harden by 70 evaporation.

8. A product comprising acetyl cellulose, triphenylphosphate and urea obtained by dissolving the same in a solvent of the acetyl cellulose and triphenylphosphate to 75 which has been added a fluid restraining agent, and then permitting the solution to dry and harden by evaporation.

9. A product comprising acetyl cellulose, triphenylphosphate and urea obtained by 80 dissolving the same in a mixture of acetone and acetylene tetrachlorid, and permitting the solution to dry and harden by evaporation.

In testimony whereof I affix my signature 85 in presence of two witnesses.

WILLIAM G. LINDSAY.

Witnesses:

HENRY J. LUCKE,  
GEO. N. KERR.